

# UNITED STATES PATENT OFFICE.

JOSIAH HUGHES AND JAMES F. MCGOWAN, OF NEW YORK, N. Y., ASSIGNORS  
TO THE IRON CLAD MANUFACTURING COMPANY, OF SAME PLACE.

## ORNAMENTAL ENAMEL-WARE.

SPECIFICATION forming part of Letters Patent No. 664,321, dated December 18, 1900.

Application filed June 21, 1899. Serial No. 721,374. (Specimens.)

*To all whom it may concern:*

Be it known that we, JOSIAH HUGHES and JAMES F. MCGOWAN, citizens of the United States, residing at New York, (Brooklyn,) in the county of Kings and State of New York, have invented certain new and useful Improvements in Ornamental Enamel-Ware, of which the following is a specification.

This invention relates to enameled ware, and it more particularly relates to the marking or ornamentation of the same.

One object of the invention is to provide improved ornamented ware having a variegated appearance, and which we have designated, for the purpose of distinguishing it from other kinds of ornamented enamel-ware, as "colonial" enamel-ware.

A further object of the invention is to provide an enameled article having an appearance more nearly resembling that of mosaic or tessellated work than anything of its kind of which we are aware.

In carrying our invention into practice the article to be enameled may be first treated in the usual manner to prepare the surface for the enamel, which usually includes the ordinary ground-coat. In some instances, if desired, this ground-coat may have incorporated with it the colored enameling materials hereinafter specified. According to the present practice, however, the article to be ornamented, having an ordinary ground-coat previously applied thereto, is then treated by being dipped or otherwise having applied thereto our improved enameling material. The body of this enameling material may be made of the usual materials well known in the art and of any suitable color, usually white or gray, and is of the consistency of paste or cream.

For the purpose of giving the variegated appearance to the article enameling materials in granulated or analogous condition are mixed with this pasty body. Each of these granulated enameling materials is prepared in a substantially similar manner to and of substantially the same kind of materials as those comprising the pasty enameling body, except for the addition of a coloring material, which is usually incorporated before the

ingredients are smelted, whereby when this takes place each enameling material assumes the color imparted to it by the coloring material. For instance, if oxid of cobalt is mixed with the enameling material it is blue, if oxid of chrome or oxid of copper is mixed therewith it is green, or if oxid of manganese or nickel, or both combined, it is brown. Other coloring materials may be used, if desired, and the coloring ingredients may be incorporated with the enameling material at other stages than that specified, if preferred or found desirable in practice. These differently-colored enameling materials when taken from the smelter are ground to the desired degree of fineness and are then mixed with the pasty enameling body, the variegated appearance of the article being secured by mixing in the proper proportions a plurality of differently-colored enameling materials with the pasty body, thus making a mixture of at least three differently-colored materials, the basic mixture or body being in a pasty condition and of one color, usually white or gray, and the two-colored materials of different colors and in a granulated condition or composed of small particles, whereby they are held mechanically suspended in the pasty body without dissolution therein, being maintained in such mechanical suspension after the mixture has been applied to the article and until the fusing of the mixture in the furnace.

In practice one colored enameling material may be of a different degree of fineness from another colored enameling material, so that the marks on the article in one color will be of a different area or larger than the marks of another color. Each colored enameling material may also have parts thereof of different degrees of fineness, so that there will be different sizes of marks of the same color on the article. For instance, if the pasty body is white and there is mixed therewith in a granulated condition a green enameling material, a brown enameling material, and a blue enameling material (the particles of each material being of the same mesh or fineness) then the marks or spots of each will be of substantially the same size, but so inter-

mixed one with another that a beautiful and highly-pleasing variegated appearance will be secured. If, however, the particles of each of the colored enameling materials are 5 of a different fineness or mesh from the others, then the marks or spots of one—as, for instance, the blue—will be of one size, while the marks or spots of the other colors will be of different sizes, but all so intermixed that 10 an article is produced having a highly-decorated variegated appearance. In practice, however, we have found that the most pleasing result is obtained by the mixing of two or more colored enameling materials, one or 15 each having parts thereof of different meshes or degrees of fineness. For instance, we mix with the pasty body—which is usually white or gray—a blue enameling material in a granulated condition, a portion of which is of a 20 different degree of fineness from another portion thereof, this also being the case with the other colored enameling materials which may be used, whereby there is provided an article which will have after being fired a variegated appearance, due not only to the different-colored enameling materials, but also due 25 to the different areas of the marks or spots of each colored enameling material. Various proportions, depending upon the character of 30 the article desired, may be used, satisfactory results having been obtained by the use of six pounds of granulated materials to fifteen pounds of pasty materials, the colored granulated materials being mixed in accordance 35 with the color which it is desired shall predominate in the article. This mixture, comprising the pasty body and the colored enameling materials thoroughly mixed with such body, is then applied to the article in any desired way—as, for instance, by dipping the 40 same therein—after which, with or without previous artificial drying, as may be best adapted for the purpose, the article is placed in the muffling-furnace, whereupon the fusing of the pasty body and of the mechanically-suspended colored enameling particles takes 45 place substantially simultaneously, so that the colored particles are fused with the body, each particle or grain, however, substantially 50 retaining its identity so far as its color is concerned, but no longer remaining in a granulated condition or in mechanical suspension, whereby the article is provided with an extremely smooth and even surface having intermixed spots or marks of different colors 55 and different areas. This fusing in the present case takes place substantially simultaneously, this being due to the formation of the enameling materials, since while the colored 60 enameling materials are in a granulated condition and the body in a pasty condition, nevertheless as the various enameling materials are made in substantially the same way, except as to the addition of the coloring materials and the grinding, they therefore fuse 65 at the same degree of heat. When the article is removed from the furnace, it will be

found that the same has a highly-decorated and pleasing variegated appearance, the marks or spots of each color blending and intermixing in such manner as to give a superior finish and an artistic and beautiful effect to the article, which appearance is materially heightened by the different areas of the various spots or marks. 75

The appearance of the article when ornamented in the manner above set forth is unlike anything we have ever seen, it more nearly resembling fine tessellated or mosaic work, this especially being the case when 80 more than two colored enameling materials are intermixed with the pasty body.

The term "color" or "colored" as used herein and in the claims is to be interpreted to mean white or black and as also including 85 shades or tints, and the term "body of one color" is to be interpreted to mean "as compared with the colors used in connection therewith, but not necessarily a uniform or solid color." 90

For the purpose of more clearly showing the distinction between the present invention and such of the prior art as have a general analogy to this invention it is deemed best to refer briefly to such prior art in so far as 95 we are aware of the same.

We are aware of a process in which the article is first highly heated and then while in such a heated condition a mixture of two or more dry enamels is sifted thereon, such dry 100 enamels being ground to a uniform fineness. This process is different from the present invention in that our article is not heated for the purpose of applying a powdered enameling material, nor are dry enamels sifted thereon, 105 nor are they of uniform fineness.

We are also aware of a process which consists in adding to a paste a granular enamel ground to a proper degree of fineness and having a fusibility greater than that of the 110 paste. This process, however, does not involve the use of a plurality of colored enameling material, or colored enameling materials of different degrees of fineness, or a mixture in which all parts thereof are fusible 115 substantially simultaneously. We are also aware of a process closely resembling the foregoing which consists in adding to a pasty 120 enameling material a second enameling material ground to a condition similar to sand and having incorporated therewith a coloring 125 material. In this instance, however, a plurality of colored enameling materials are not used in connection with the pasty material, nor do such enameling materials have different degrees of fineness.

We are also aware of a process in which after the article is treated to one coat of enameling material it is treated to a thin glaze composed of any coloring material which can 130 be made to remain mechanically suspended a short time in water and of such a character that the glaze will separate and coagulate in irregular spots. In this process the coloring

material is evidently of a solvent character and is not adapted to remain mechanically suspended in an enameling material until the fusing of the article, nor are the coloring 5 enamels of different degrees of fineness. In fact, the coloring-matter used must be such as will permit the glaze to be a liquid, and this coloring-matter is not an enameling material, but merely an ingredient adapted to 10 give color to the glaze, nor does the article have when produced a mosaic or tessellated appearance. Moreover, in the present process the enameling mixture does not coagulate in irregular spots, nor are such spots of varying 15 thickness, thus impairing the smoothness and uniformity of the surface of the article.

In conclusion we are also aware of other processes in which, for instance, oxid of iron 20 is mechanically suspended in an enameling material and is infusible therein; but none of them, however, have the characteristics and advantages of the present invention, in which a plurality of colored enameling materials 25 each having portions of different degrees of fineness are mixed in a pasty enameling body and remain mechanically suspended therein until the fusing of the whole, all parts of which take place substantially simultaneously, whereby an improved ornamental article is provided.

Having described our invention, we claim—

1. Enameled ware having a mosaic, tessellated, or variegated appearance, the surface 35 of which comprises a body of enamel having incorporated and fused therein an enameling material of different colors.

2. Variegated enameled ware having a surface comprising a body of one color, having 40 incorporated and fused therewith a plurality

of enameling materials of a character to form spots or marks, and each such material of a color different from such body and from each other.

3. Variegated enameled ware having a surface comprising a body of one color, having 45 incorporated and fused therein a plurality of enameling materials of a character to form spots or marks, and each such material of a color different from such body, and from each 50 other, the spots or marks of one color having areas different from the spots or marks of its companion color or colors.

4. Variegated enameled ware having a surface comprising a body of one color, having 55 incorporated and fused therewith a plurality of enameling materials of a character to form spots or marks; and each such material of a color different from such body and from each other, and the spots or marks of each one of 60 the colors having different areas.

5. Enameled ware having a mosaic, tessellated, or variegated appearance, the surface of which comprises a body of enamel having 65 incorporated and fused therewith an enamel- ing material of different colors and areas.

6. Variegated enameled ware having a surface comprising a body of one color, having incorporated and fused therewith an enamel- 70 ing material of different colors to form spots or marks of different areas, some of such spots or marks having areas similar to that of a speck or pepper-grain; and others of such spots having varying and materially increased areas.

JOSIAH HUGHES.  
JAMES F. MCGOWAN.

Witnesses:

C. A. WEED,  
J. S. CLARK.